

## UNITED STATES PATENT OFFICE

1,960,895

## PROCESS FOR PREPARING METAL ARTICLES

Willis H. Castner, Cornwall, Pa., assignor to Bethlehem Steel Company, a corporation of Pennsylvania

No Drawing. Application February 21, 1930,  
Serial No. 430,449

2 Claims. (Cl. 143—4)

My invention relates to a process for preparing metal articles which are to be of definite, predetermined shape or dimensions.

My invention relates to methods wherein the metal articles are to be subjected after their formation to a heat operation at such temperatures as would normally oxidize the metal.

My invention consists in forming the article, coating with a non-oxidizable metal, and then heat treating at temperatures which would oxidize the article but for the protective coating.

My invention can probably be best illustrated by giving a specific example. Obviously the protection sought is not to be limited to this specific illustration. As such example, let us take the manufacture of threaded bodies such as screws or bolts.

A ferrous metal blank is prepared of the desired form and dimensions and is then machined to produce threads of the desired character and dimensions. These screws, or at least the threaded portions thereof, are then placed in an electrolyte containing a chromium salt and electro plated to cover the threaded portions or such portions of the screw as it is desired to protect, with a very thin coating of chromium say of a thickness of from two to three ten-thousandths of an inch.

The screws are then subjected to a heat treatment to improve the mechanical characteristics of the metal of such screws. They are heated above the critical range and quenched in oil, water or other suitable quenching medium. The screws are then "drawn", that is they are held at an elevated temperature but such temperature as is below the critical range until the desired microstructure in the screw is obtained.

Such a treatment, if it were not for the chromium coating, would inevitably result in a more or less deep oxidation of the metal of the screw. For the threaded portion of the screw this would be especially detrimental as such oxidation would not only alter the "fit" of the screw because of the change in form and dimension, but the scale which might burn fast to the metal would be very troublesome. The chromium coating, which is sufficiently thin not to substantially alter the desired thread form and dimension, effectively prevents any substantial oxidation.

The chromium plating may be effected by any of the well known processes of the art.

While I have specified chromium and while chromium is especially advantageous, it is obvious that my invention contemplates the use

of any protective material which will effectively resist oxidation.

Obviously the protective coating must either be so thin as to be negligible so far as in its effects upon size and dimensions of the body being treated, or an allowance must be made for the thickness of the coating in the formation of the body prior to the coating.

By the expression "heat treatment" in the claims I intend to include any treatment at such temperatures as would cause oxidation of the metal of which the body is composed. For example, in addition to heating for hardening or for drawing, as above given operations such as normalizing, and the like obviously are also to be included.

The essential thought of the invention is the use of chromium or some other protective coating before the heat treatment so that such heat treatment will have practically no effects upon the definite, predetermined form and dimensions desired in the article.

Having thus described my invention what I claim and desire to secure by Letters Patent is:

1. In a process for preparing ferrous articles to have definite, predetermined form and dimensions, the steps of machining the article to the desired finished form and dimensions, covering with a coating of chromium of negligible thickness and heat treating at temperatures and under conditions which would oxidize the surface of the article but for the chromium coating.

2. In a process for manufacturing threaded articles to have threads of definite, predetermined form and dimensions, the steps of giving the article threads of the desired finished form and dimensions by machining, coating the threaded portion of the article with a coating of chromium sufficiently thin to inappreciably affect the form and dimensions of the thread and heat treating the articles at temperatures and under conditions which would oxidize the threads but for the chromium coating.

WILLIS H. CASTNER.

100

105

110